

## UNITED STATES PATENT OFFICE

2,240,300

## MANUFACTURE OF PHONOGRAPH RECORDS

James H. Hunter, Lansdowne, Pa., assignor to  
Radio Corporation of America, a corporation of  
Delaware

No Drawing. Application June 30, 1937,  
Serial No. 151,312

3 Claims. (Cl. 204—5)

This invention relates to the phonograph record art, and more particularly to a method of preparing recording waxes for the electro-deposition of a metallic coating thereon which, when stripped from the wax, constitutes a master matrix.

In the production of phonograph records, after the original recording has been made in a wax blank, the wax record is coated with a metalizing powder and subsequently electro-plated with a suitable metallic deposit which, after being removed from the wax and backed up by a copper or other metal backing, serves as the master matrix. The metalizing powder is necessary in order to make the surface of the wax electro-conductive. Up to the present time, various metalizing powders have been used in making the surface of the wax or other similar non-conductive body conductive, and all of them, so far as I am aware, have depended solely on the tackiness of the body to hold the powder to the surface thereof. Inasmuch as the tackiness of the wax varies greatly with temperature, being reduced considerably when the wax is cold, reliance solely upon the tackiness of the wax constituted a great disadvantage.

The primary object of my invention is to provide an improved method of applying the electro-conductive powder to the surface of the wax to cause the same to adhere thereto.

More specifically, it is an object of my invention to provide an improved metalizing powder which will adhere strongly to the surface of the wax record regardless of the temperature thereof.

I have found, in accordance with my invention, that by the addition of a very small amount of a fatty acid, such as stearic acid, oleic acid, lard or similar materials, to the metalizing powder, the adhesion thereof to the recording wax is greatly improved, and this results in an improvement in the electro-depositing operation. I have also found that even when a small amount of tack producing material is incorporated with the metalizing powder the difficulties experienced in cold weather are no longer encountered. As an example of the effectiveness of my improved metalizing powder, I have found that the addition of approximately 0.1% by weight of stearic

acid to a bronze powder made up of 90% copper and 10% zinc imparted to the powder very great adhesive characteristics. This also gave a much more uniform layer of electro-deposited metal.

5 Although I have mentioned a few of the materials which effectively produce tackiness in the metalizing powder, it will be readily apparent to those skilled in the art that many other similar materials may be used as well. Also, I wish it to be understood that the percentage of fatty acid added to the metalizing powder is merely illustrative and not in any way limiting. Since the specific tack producing material employed and the quantity thereof may be varied over a wide range, I desire that my invention shall not be limited except insofar as is made necessary by the prior art and by the spirit of the appended claims.

I claim as my invention:

20 1. The method of forming a phonograph record matrix which comprises preparing an original wax phonograph record, applying to said wax record a conductive powder having incorporated therein approximately 0.1 percent by weight of a fatty composition selected from the group consisting of stearic acid, oleic acid and lard, electrodepositing a layer of metal over said powder, and finally separating said electrodeposited metal layer from said wax record.

25 2. The method of forming a phonograph record matrix which comprises preparing an original wax phonograph record, applying to said wax record a conductive powder having incorporated therein stearic acid in an amount of approximately 0.1 percent by weight, electrodepositing a layer of metal over said powder, and finally separating said electrodeposited metal layer from said wax record.

30 3. The method of forming a phonograph record matrix which comprises preparing an original wax phonograph record, applying to said wax record powdered bronze having incorporated therein stearic acid in an amount of approximately 0.1 percent by weight, electrodepositing a layer of metal over said powder, and finally separating said electrodeposited metal layer from said wax record.

JAMES H. HUNTER.